

1

2,788,301

## METHOD OF COATING STEEL AND PRODUCT THEREOF

Elton B. Moore, Calumet City, and Elliot S. Nachman, Park Forest, Ill., assignors to La Salle Steel Co., Hammond, Ind., a corporation of Delaware

No Drawing. Application June 15, 1955,  
Serial No. 515,794

6 Claims. (Cl. 148—4)

This invention relates to the working of steel as by drawing steel bars, rods, wires or tubes to effect reduction in cross-sectional area and it relates more specifically to the treatment of steel in working or drawing to improve the surface finish of the steel, to reduce the load required to effect the desired reduction in cross-sectional area and to improve the physical and mechanical properties of the steel.

This application is a continuation-in-part of our pending application Ser. No. 293,435, filed June 13, 1952, entitled "New and Improved Steel Products and Methods for Producing Same," now abandoned.

It is an object of this invention to provide a method for improving the surface finish of steel as an incidence to the working of the steel for effecting a reduction in cross-sectional area and it is a related object to treat the surface of the steel in advance of working to effect reduction in cross-sectional area with a material that reacts with the conditions existing to produce a new and improved surface finish on the steel and which also reduces the load required to effect the reduction in cross-sectional area.

More specifically, it is an object of this invention to coat the steel prior to working to effect reduction in cross-sectional area, as by advancing the steel in the form of a bar or rod through a draw die, wherein the coating reacts to produce a bright, shiny and smooth surface layer on the steel and which acts as a lubricant to reduce the load required to effect the desired reduction in cross-sectional area wherein the reduction in pull load is greater than heretofore secured by conventional lubricants of the type heretofore employed.

In the aforementioned copending application, of which this is a continuation-in-part, description has been made of a new and improved metallurgical process for producing a bright and shiny surface layer on steel as an incidence to the working of the steel to effect reduction in cross-sectional area, as by drawing the steel through a draw die. The invention is described with reference to development of the desired results with a non-austenitic steel having a pearlitic structure in a matrix of free ferrite, but it is believed that the invention in the development of the desired characteristics is available also with other steels and alloy steels.

In accordance with the teaching of the aforementioned application, the new and improved surface finish is developed when the steel, heated to a temperature in excess of 300° F. and preferably to within the range of 300–1100° F., is advanced through a draw die to effect reduction in cross-sectional area while coated with molybdenum disulphide prior to such working to effect reduction.

It has now been found that the improvements secured by working the steel at an elevated temperature to effect reduction in cross-sectional area with molybdenum disulphide present as a coating on the steel are available also when the steels are coated with other compounds, such for example as cadmium iodide, copper bromide,

2

tungsten sulphide, silver sulphate and the like. While these compounds are somewhat unlike molybdenum disulphide and not equivalent thereto in the general sense, it appears that these other compounds have a similar 5 layer, lattice-type structure as molybdenum disulphide which enables reaction on the steel under the pressure and temperature conditions existing in the draw die to produce a finish which is similar in appearance and structure but of necessity different in composition than 10 that secured with molybdenum disulphide.

It has been found further that the presence of molybdenum disulphide or the other compounds on the surfaces of the steel results also in a marked reduction in the load required to effect the desired reduction in cross-sectional area of the steel. As such the molybdenum disulphide and other compounds function additionally as a lubricant for the steel when processed through a metal draw die or otherwise worked to effect reduction in cross-sectional area. Reduction in pull load 20 is particularly effective with the use of molybdenum disulphide when the steel drawn is heated to a temperature in excess of 300° F. and preferably within the range of 300–1100° F.

The invention herein will be described with particular 25 reference to the use of molybdenum disulphide as the substance applied, preferably in the form of a dry powder, to the surface of the steel for reaction to develop the desired results under the temperature and pressure conditions existing, but it will be understood that the other 30 compounds having a layer, lattice-type structure, such as previously named, may also be used.

The molybdenum disulphide reacts on the steel surface 35 differently than other metal salts which might previously have been used as metal lubricants, such for example as lead sulphide. The difference between molybdenum disulphide and lead sulphide, for example, is particularly noticeable from the standpoint of appearance which each imparts to the finished steel as it emerges from the draw die and afterwards and the difference is also noticeable 40 from the standpoint of pull loads in pounds required to effect equivalent reductions in similar steels under similar conditions, especially in drawing steel heated to an elevated temperature in excess of 300° F. Differences are 45 also noticeable from the standpoint of the finish which is secured on the steel by way of surface smoothness and the other characteristics of the drawn steel.

The amount of molybdenum disulphide applied to the 50 surface of the steel is not critical as long as an amount of molybdenum disulphide is present on the surface sufficient to form a substantially continuous monomolecular film comprised of the reaction product that is formed between the molybdenum disulphide and the steel at the surface. An excess of molybdenum disulphide may be 55 present on the steel but the depth of the new and improved surface layer having a bright metallic and silver-like finish is not substantially increased and therefore the presence of such excesses are of no apparent value.

When processed in accordance with the practice of this 60 invention, the steel issuing from the draw die is characterized by having a smooth and permanent bright metal finish. The surface appears to be highly resistant to deterioration, dulling or attack by elements normally existing in the atmosphere. It is possible by taking abnormally heavy drafts with appropriate die practice, to 65 produce an improved surface without heating the metal to an elevated temperature. However, the unexpected reductions in drawing load are secured mainly when drawing with molybdenum disulphide on the surface of the steel which has been heated to an elevated temperature in 70 excess of 300° F. When compared directly to lead sulphide or to sodium bismuthate and the like, the molybdenum disulphide present on the surface of the steel is

effective also to reduce the drawing load required to effect reduction in cross-sectional area as will hereinafter appear.

The following will illustrate the vast improvement secured by the use of molybdenum disulphide as a dry powdered lubricant for steel used in metal drawing operations as compared to such materials as lead sulphide, antimony sulphide, sodium bismuthate, or conventional oil type lubricant, referred to hereinafter as the Nox-rust compound.

#### EXAMPLE 1

Two austenitic steels having the following composition were subjected to a series of identical processing steps:

| Material | C   | Mn   | P    | S    | Si  |
|----------|-----|------|------|------|-----|
| C-1018   | .16 | .71  | .010 | .030 | .25 |
| C-1144   | .44 | 1.52 | .018 | .310 | .29 |

The following is the procedure which was used for 20 making the comparison:

5/8 inch diameter bars of C-1018 and C-1144 steels were drawn at 1/16 inch draft to a 1/16 inch diameter (1) at room temperature after the prescribed lubricant had been applied dry; (2) at 400° F. with the lubricant applied dry (a) before heating and (b) after heating but before drawing. The steel was drawn at the rate of 25 feet per minute.

The results which were secured with the two different steels drawn under the described conditions are tabulated 30 as follows:

#### DRAWING AT ROOM TEMPERATURE

| Lubricant             | C-1018                 |                             | C-1144                 |                             |
|-----------------------|------------------------|-----------------------------|------------------------|-----------------------------|
|                       | Average Pull in Pounds | Appearance                  | Average Pull in Pounds | Appearance                  |
| Molybdenum disulphide | 8,590                  | Chrome-like bright metallic | 10,845                 | Chrome-like bright metallic |
| Lead sulphide         | 9,735                  | Mottled gray                | 13,755                 | Mottled gray                |
| Antimony sulphide     | 8,590                  | do                          | 10,845                 | Do                          |
| Sodium bismuthate     | 9,735                  | Orange gray                 | 13,300                 | Orange gray                 |
| Nox-Rust              | 8,025                  | Mottled gray                | 10,845                 | Mottled gray                |

#### DRAWING LUBRICATED STEEL AT 400° F.

|                       |       |                             |        |                             |
|-----------------------|-------|-----------------------------|--------|-----------------------------|
| Molybdenum disulphide | 6,015 | Chrome-like bright metallic | 8,590  | Chrome-like bright metallic |
| Lead sulphide         | 8,590 | Mottled gray                | 12,685 | Mottled gray                |
| Antimony sulphide     | 9,165 | do                          | 8,590  | Do                          |
| Sodium bismuthate     | 8,020 | Orange gray                 | 10,270 | Orange gray                 |

#### DRAWING AT 400° F. WITH LUBRICANT APPLIED AFTER HEATING

|                       |        |                             |                            |                             |
|-----------------------|--------|-----------------------------|----------------------------|-----------------------------|
| Molybdenum disulphide | 6,585  | Chrome-like bright metallic | 9,735                      | Chrome-like bright metallic |
| Lead sulphide         | 13,755 | Mottled gray                | 15,450                     | Mottled gray                |
| Antimony sulphide     | Broke  |                             | Lack of proper Lubrication |                             |
| Sodium bismuthate     | 9,735  | Orange gray                 | 9,735                      | Orange gray                 |
| Nox-Rust              | 8,310  | Mottled gray                | 8,595                      | Mottled gray                |

The surface appearance of a drawn steel bar represents an important consideration which controls the selection of a lubricant because it is desirable to have the surface of the drawn bar free of defects not only from hot mill rolling, such as laps and seams, but also free of scratches and galling due to lack of lubrication or from improper lubrication. From the data which has been developed as set forth in the foregoing tables, it will be seen that steels drawn with molybdenum disulphide as a lubricant are characterized by having a bright, shiny, smooth metallic surface approaching a chrome-like appearance when compared with the relatively dull, mottled gray appearance visible on the surfaces of the same steels drawn with other lubricants such as lead sulphide, sodium bismuthate, antimony sulphide, and conventional oil base lubricants.

A distinctively different reaction occurs in the use of molybdenum disulphide as the material on the surface of the steel to be drawn as distinguished from the presence

of other materials conventionally employed as lubricants or for surface treatment. This reaction not only results in reduced friction between the die and metal drawn but also produces a plate-like deposit which is quite unlike any deposit heretofore observable. By the use of appropriate pressures and temperatures, the layer structure is produced which is strongly adherent and appears to be an integral part of the surface of the drawn steel part.

Because of the reaction which appears to take place to 10 form a smooth surface on the steel in the draw die or for whatever other unknown reasons or reaction, it has been found that the pull load required to effect a reduction in cross-sectional area is less in the use of molybdenum disulphide than for other lubricants especially when 15 operating on steel heated to an elevated temperature.

By comparison with conventional lubricants, the pull load with molybdenum disulphide was less in every instance than the pull load with other materials at the same temperature, with the same steels, at the same amount of reduction. For example, the pull load with molybdenum disulphide at 500° F. was as much as 50 percent less than the pull load required with a similar reduction with the same steel and effected with lead sulphide, and the pull load with molybdenum disulphide was never more than 25 percent less than the pull load for lead sulphide.

The following example will illustrate the improvements which are secured in appearance of the steels drawn at various temperatures ranging from room temperatures up to about the lower critical temperature for the steel composition:

60 The following data was developed with steel having the following composition:

0.48 percent carbon  
1.50 percent manganese  
0.03 percent phosphorus  
0.27 percent sulphur  
0.30 percent silicon  
0.005 percent nitrogen

In developing the results, hot rolled steel bars of 5/8 inch in diameter were drawn through a die and given a 1/16 inch reduction. The bars were advanced to the draw die while heated to temperatures of 75, 300, 500, 700, 900 and 1200° F. respectively. Before advancing the heated bars through the draw die, powdered molybdenum disulphide was wiped onto the surfaces of the steel to

function as a lubricant and as a reactant to produce a bright and highly resistant finish on the steel surface.

The following table compares the surface finish of the steels drawn through the die at various temperature levels with a coating of molybdenum disulphide on the surfaces thereof and without the use of other lubricants:

*Effect of drawing at elevated temperatures on surface finish*

| °F.                            | 75°   | 800°        | 500°          | 700°          | 900°          | 1,200° |
|--------------------------------|-------|-------------|---------------|---------------|---------------|--------|
| Surface Finish in Micro inches | 20-30 | 20          | 15            | 6             | 10            | 10     |
| Surface Appearance             | Matte | semi-bright | chrome bright | chrome bright | chrome bright | Matte  |

It will be apparent from the foregoing that the non-austenitic steels having a pearlitic structure in a matrix of free ferrite permit the use of molybdenum disulphide as a drawing lubricant for steels and that when the steel is drawn through the die at elevated temperatures between 300° and 1100° F., marked reduction in surface roughness and a bright surface finish are substantially permanently formed on the surface of the drawn metal thereby to improve the appearance and characteristics of the steel and eliminate the additional steps heretofore required to obtain a surface finish and to protect the finish from attack or deterioration.

The method of heating to raise the steel to the desired temperature levels for drawing is unimportant. Use is made of conventional means such as an oil bath, gas fired furnace, electrical heating means or the like. In the event that the technique described and claimed in the copending application of Elliot S. Nachtman, Ser. No. 286,039, filed May 3, 1952, now abandoned, is employed to prepare the steel surface for drawing, as by the application or treatment with molten salts, temperature of the desired level may be introduced by the molten salts and the molybdenum disulphide embodied as an ingredient therein to produce the desired finish on the steel surface. It is preferred, however, to apply the molybdenum disulphide in accordance with the practice herein subsequent to the salt treatment, with or without the removal thereof.

### EXAMPLE 3

#### Steel composition:

0.17 percent carbon  
0.75 percent manganese  
0.03 percent phosphorus  
0.04 percent sulphur  
0.08 percent silicon  
0.005 percent nitrogen

5/8 inch hot rolled steel of the above composition, which is a steel of the non-austenitic type having a pearlitic structure in a matrix of free ferrite, was heated to a temperature of 900° F. in a gas fired furnace and advanced continuously through a drawing die to secure a 19 percent reduction in cross-sectional area. One group of bars were drawn through the die with a normal oil base lubricant applied to the surface thereof while another group were coated in advance of passage through the die with molybdenum disulphide dispersed in 5-10 percent concentrations in a grease composition.

The surface finish on the drawn steel not having molybdenum disulphide applied to the surface thereof was matted and dulled and required a subsequent grinding operation to increase its luster and then had to be wrapped in a special treated paper to protect the surface finish against rusting or deterioration by elements normally existing in the atmosphere. On the other hand, the surface finish on the steel drawn through the die under the same conditions but with molybdenum disulphide on the surface thereof had the appearance of bright chrome and resisted deterioration or attack. For all practical purposes, it appears as though the salt had been reacted under the heat and pressure existing in the draw die to

form a new compound of the molybdenum disulphide or reduce the compound to molybdenum metal or an alloy thereof with the steel but in any event, the new substance is strongly anchored and embedded in the surface of the drawn steel to become a permanent part thereof.

It is believed that this is the first time that molybdenum

disulphide has been used to produce a bright and protective surface of this character on steel. It is believed that this is the first time that molybdenum disulphide has been used to reduce the pull load required to draw steel through a draw die to effect reduction in cross-sectional area.

It will be apparent from the foregoing that the combination of pressure and temperatures available during drawing steel to effect reduction in cross-sectional area provide conditions by which these new and desirable results are developed. Reaction sufficient to develop an improved surface finish on the steel may be secured by the use of molybdenum disulphide without preheating the metal to an elevated temperature but the brightness is not as good as that secured with steel heated to an elevated temperature. The pull load is also reduced by the use of molybdenum disulphide as a lubricant when compared with the use of other salts such as lead sulphide, sodium bismuthate and the like to lubricate the surface of steel in a drawing operation.

As used herein, the term "surface roughness" is an indication of the smoothness of the formed surface taken by a profilometer readable in terms of micro inches.

It will be understood that the use of molybdenum disulphide or other compounds having a layer-lattice-type structure such as cadmium iodide, copper bromide, tungsten sulphide and silver sulphate as a lubricant and as a material to develop improved surface characteristics on metal and to reduce drawing loads is not limited to use with non-austenitic steels of the type described. It is believed that the application of molybdenum disulphide as a lubricant and as a surface treating composition concurrently to improve the character of the surface finish and reduce pull load is applicable to other steels and alloys of steel and that such other uses may be made without departing from the spirit of the invention, especially as defined in the following claims.

We claim:

1. The method of treating steel to produce a smooth surface layer of improved brightness comprising working the steel to effect a reduction in cross sectional area at a temperature above 300° F. but below the lower critical temperature for the steel composition and with a coating of molybdenum disulphide on the surface thereof.
2. The method of processing steel of the non-austenitic type having a pearlitic structure in a matrix of free ferrite to improve the characteristics thereof comprising the steps of drawing the steel through a drawing die while the steel is heated to a temperature within the range of 300-1100° F. and with a coating of molybdenum disulphide on the surface thereof.
3. The method of processing steel of the non-austenitic type to improve the characteristics thereof comprising the steps of heating the steel in a solid integral mass to a temperature above 300° F. but below the lower critical temperature for the steel composition, coating the heated steel with molybdenum disulphide and then working the coated and heated steel at a temperature above 300° F. whereby reaction takes place to form a bright and permanent metal finish on the steel surface.

4. The method of processing steel of the non-austenitic type comprising the steps of heating the steel to a temperature above 300° F. but below the lower critical temperature for the steel composition, coating the steel surface with molybdenum disulphide and then drawing the steel through a drawing die to effect reduction in cross sectional area while heated to the elevated temperature.

5. The method of processing steel of the non-austenitic type comprising the steps of heating the steel in advance of drawing to a temperature between 300° and 1100° F., applying a molybdenum disulphide powder to the surface of the heated steel and then drawing the steel through a drawing die to effect reduction in cross sectional area while heated to the elevated temperature.

6. The method of processing steel of the non-austenitic type comprising the steps of coating the steel in advance of drawing with a composition containing molyb-

denum disulphide, and then advancing the steel through a drawing die to effect reduction in cross sectional area while the steel is at a temperature above 300° F. but below the lower critical temperature for the steel composition.

5

## References Cited in the file of this patent

## UNITED STATES PATENTS

|           |          |               |
|-----------|----------|---------------|
| 2,280,886 | Brace    | Apr. 28, 1942 |
| 2,361,211 | Zimmer   | Oct. 24, 1944 |
| 2,400,866 | Kronwall | May 21, 1946  |
| 2,588,234 | Henricks | Mar. 4, 1952  |

## OTHER REFERENCES

15 Alloy Metals Review, vol. 7, No. 51, March 1949 (pp. 2-8).